

Aug. 22, 1950

W. STUBBLEBINE

2,519,410

HARD SURFACE FLOOR AND WALL COVERING

Filed Nov. 30, 1944

FIG. 1



FIG. 2



INVENTOR.

W. Stubblebine  
by  
Walter + George

## UNITED STATES PATENT OFFICE

2,519,410

## HARD SURFACE FLOOR AND WALL COVERING

Warren Stubblebine, Lancaster, Pa., assignor to Armstrong Cork Company, Lancaster, Pa., a corporation of Pennsylvania

Application November 30, 1944, Serial No. 565,907

1 Claim. (Cl. 154—49)

**1** This invention relates to hard surface floor or wall coverings, and more particularly, to a hard surface floor or wall covering including a unitary, partible, felted, fibrous stratum having an alkyd resin uniformly dispersed throughout the mass of the fibrous stratum in an amount sufficient to render such stratum substantially water-resistant and to strengthen said stratum to prevent its separation into laminae when exposed to traffic conditions, but insufficient to completely fill the interstices thereof whereby, when the covering is adhesively secured to a base, the stratum may be subsequently ruptured to permit removal of the covering from the base.

It is well-known that floor coverings including a saturated fibrous backing are extremely difficult to remove from a base when adhesively secured thereto. Various proposals have been offered heretofore to remedy this difficulty which is inherent in the use of such types of floor covering. For example, it has been proposed to provide the saturated felt backing with a rupturable coating in order to permit removal of the covering from a base to which it is adhesively secured. That is, when the covering is adhesively secured in place and tensile forces are applied to remove the covering, the coating ruptures to permit removal of the covering from the base. This procedure is extremely difficult to carry out commercially. Under commercial conditions, it is extremely difficult to formulate and maintain a coating within required limits of rupturability, and in many cases, the coating is too weak so that the covering is separated from the base when exposed to traffic while in other cases, the coating is stronger than the saturated felt so that attempted removal ruptures the backing rather than the coating, leaving an unsightly mass of felt on the base which is extremely difficult to remove for the saturant prevents the penetration of water to the adhesive.

It has also been proposed to render floor coverings of this type removable by differentially saturating the felt backing. That is, the portion of the felt backing adjacent the wear surface of the covering contains a large amount of saturant while the portion of the backing adjacent the base contains saturant in an amount considerably smaller than the amount of saturant contained in the portion of the backing adjacent the wear surface. The theory proposed is excellent while the commercial application of the theory is difficult is not well-nigh impossible. Under commercial conditions, it is impossible to differentially saturate a felt sheet

**2** satisfactorily. Either too great an amount of saturant is disposed in a portion of the sheet which should carry a small amount of saturant or insufficient saturant is disposed in the portion of the sheet adjacent the wear surface. Accordingly, such proposals, while theoretically possessing merit, are impracticable from a commercial point of view.

The chief object of my invention is to provide a floor or wall covering of the type described above in which the disadvantages involved in commercial production are obviated. A further object of my invention is to provide a floor or wall covering including a felt backing containing alkyd resin uniformly permeating the mass of the fibrous backing. A further object is to provide an easily removable floor or wall covering including a unitary, partible, felted, fibrous stratum. A still further object is to provide a hard surface floor or wall covering which includes a unitary, partible, felted, fibrous stratum carrying an alkyd resin dispersed substantially uniformly therethrough in an amount sufficient to render the fibrous stratum substantially water-resistant and to strengthen the fibrous stratum to prevent its separation into laminae when exposed to traffic conditions.

This invention relates to a hard surface floor and wall covering which includes a unitary, partible, felted, fibrous stratum, the fiber constituents of said stratum being substantially uniformly felted throughout the thickness thereof, and an alkyd resin uniformly permeating the fibrous stratum, said resin being dispersed substantially uniformly throughout the mass of the fibrous stratum in an amount sufficient to render the fibrous stratum substantially water-resistant and to strengthen said stratum to prevent its separation into laminae when exposed to traffic conditions, but insufficient to completely fill the interstices thereof, whereby when the covering is adhesively secured to a base, the stratum may be subsequently ruptured to permit removal of the covering from the base.

45 The attached drawing illustrates a preferred embodiment of my invention, in which

Figure 1 is a sectional view of the floor covering of my invention adhesively secured to a base; and

50 Figure 2 is a diagrammatic view illustrating the process of manufacture of the floor covering of my invention.

Referring to the drawing, there is disclosed a unitary hard surface floor or wall covering 2 composed of a wear-resistant surface 3 integrally

united with a fibrous stratum or backing 4. Preferably, wear surface 3 is composed of a siccative oil-resin gel, fillers, and pigments as is customary in the manufacture of linoleum compositions. It will be understood it may comprise a wear-resistant paint coating if desired.

The fibrous stratum 4 is composed of a mass of fibers uniformly felted throughout the thickness thereof and is permeated by an alkyd resin uniformly dispersed throughout the mass thereof. The alkyd resin is present in an amount sufficient to render the fibrous stratum substantially water-resistant and to strengthen said stratum to prevent its separation into laminae when exposed to traffic conditions. The amount of alkyd resin carried by stratum 4 is insufficient to completely fill the interstices of the fibrous stratum, whereby when the covering is adhesively secured to a base, the stratum may be subsequently ruptured to permit removal of the covering from the base.

Preferably, the alkyd resin is formed by the condensation polymerization of an aliphatic dibasic acid containing fourteen to thirty carbon atoms, castor oil, and glycerol; for example, castor oil may be broken down into various dibasic acids, and such acids, the castor oil residue and glycerol reacted to form the alkyd resin. In this case, the dibasic acid replaces phthalic anhydride ordinarily used to form alkyd resins. It will be understood that the alkyd resin is not in "cured condition" when it is dispersed throughout the mass of the fibrous stratum since a substantially completely polymerized resin would not be capable of uniformly permeating the mass of the fibrous stratum. I prefer to use an alkyd resin, such as "Duraplex AL-210," though any oil-modified alkyd resin may be used if it does not become too hard when cured or substantially completely polymerized.

The floor covering 2 is secured to a base 5 by a layer 6 of any suitable adhesive composition. When it is desired to remove the covering 2 from the base, application of tensile forces to the covering ruptures the fibrous stratum 4, permitting removal of the covering from the base. Only a thin layer of felt remains on the base and such small amount of felt may be easily and quickly removed by the application of a solvent, for example, water, if a water type adhesive be used, since the impregnant does not fill the interstices of the felt and the solvent can quickly and readily penetrate the felt to weaken the adhesive bond.

The fibrous stratum carrying an alkyd resin as contemplated by my invention in non-staining; a seal coating is unnecessary to improve its physical properties and appearance. The elimination of seal coatings considerably decreases the cost of manufacture, particularly when the wear surface is composed of a wear-resistant paint, since bleeding of the impregnant into the wear surface cannot occur. It will be understood, of course, if desired, a seal coat may be applied, but as pointed out above, this is not necessary.

In the manufacture of the floor covering of my invention, any usual flooring felt may be impregnated with the alkyd resin described above. A roll of flooring felt 7 is coated with a coating of alkyd resin 8 by means of an applicator roll 9 which applies the resin to one side of the felt sheet. The felt sheet carrying the alkyd resin is then warmed by passing it over heated drums 10 and is formed into rolls 11 while warm and permitted to remain in rolled condition for about twenty-four hours thus permitting the alkyd resin to permeate substantially uniformly

throughout the fibrous sheet. Preferably, the alkyd resin is maintained at a temperature of 180° to 220° F. when it is applied to the felt sheet. After the resin has permeated substantially uniformly throughout the fibrous sheet, it is carried into a stove or oven 12 and the alkyd resin is cured at a temperature of 175° to 200° F. Such temperatures are preferable, but it will be understood higher temperatures reduce the time required for complete conversion of the resin. The cured resin is tough and strong.

The wear coating 3 may be integrally united with the fibrous stratum as is customary and well-known in the floor covering industry. If desired, such wear surface may be cured or stoved without affecting in any way the rupturable characteristics of the fibrous backing. The fibrous backing should contain the alkyd resin in an amount falling within the range of 25% to 30% of the weight of the dry felt. Such resin, as pointed out above, is uniformly dispersed throughout the mass of the fibrous sheet and renders the fibrous sheet substantially water-resistant and strong enough to resist severe traffic conditions, but is insufficient to prevent ready removal of the covering from a base to which it is adhesively secured.

In my experiments, I have determined certain definite limits of cohesion within which the strength or resistance to tensile forces of the fibrous stratum must fall in order to obtain ready removability. I have determined that limits of cohesion of 3 to 30 pounds are satisfactory, but limits of 6 to 30 pounds are preferred. With greater tensile resistance than 30 pounds, the fibrous stratum is resistant to a degree to prevent ready removability. With tensile resistance less than 3 pounds, it is dangerously weak and may be separated into laminae by severe traffic and excessive wear. For that reason, a minimum of 6 pounds is preferred. The "pull" test, hereinafter referred to as the Scott test used to establish these limits, may be carried on in the following manner:

To one side of a strip of wood 6" long and 2" wide, a thin layer of linoleum cement or paste is applied using a notched doctor blade to apply the paste or cement evenly over the entire surface. To the paste or cement is immediately applied a strip of the covering to be tested 8" long and 2" wide, one end of which is placed flush with one end of the strip of the wood, the other end extending freely beyond the wood strip. After rolling to obtain a satisfactory bond between the wood and the covering, the sample is maintained at normal room temperature for approximately four days to dry the paste or cement. The resistance of the fibrous stratum to tensile forces is determined by placing the sample in a Scott tensile strength machine at right angles to the direction of the forces to be exerted. The strength of the forces recorded as the covering is removed from the wood strip measures the resistance of the fibrous stratum to tensile forces.

While the present invention has been described as particularly adapted to the manufacture of so-called felt base and linoleum-like floor or wall coverings, it is likewise adapted for use in the production of coverings, such as industrial flooring which comprises a saturated felt base or body carrying an asphaltic coating as a wearing surface; floor coverings in which the fibrous stratum itself may form the wearing surface, or any similar floor coverings which include a partible

fibrous stratum, such as asphalt-saturated felt underlayment for resilient tiles and the like.

A building structure embodying my invention may be formed in the following manner: The base is prepared to receive a covering; that is, it is cleaned and levelled so that it presents a clean, dry, substantially smooth surface. A layer of adhesive is spread evenly over the base; the hard surface covering is laid thereon before the adhesive is dry and firmly pressed thereagainst as by rolling, placing heavy sand bags thereover, or the like. When the adhesive has dried, the covering is securely attached to the base.

When it is desired to remove the covering, the fibrous stratum may be readily ruptured by exerting tensile forces on the structure. The felt splits, or separates into laminae, leaving a thin layer or lamina of the alkyd resin impregnated felt secured to the base while the major portion of the fibrous stratum is removable with the wearing surface. When the covering is removed, the base may be readily placed in condition to receive a new covering by washing away the minor portion of felt and adhesive remaining thereon and following the process described above.

The floor or wall covering of my invention possesses definite removable features which are not affected by the temperatures or length of time required for maturing the wear surface. The rupturable fibrous stratum is inexpensive and satisfactorily resistant to traffic conditions while retaining its rupturable characteristics. It is inexpensive and is quickly and easily applied to form the decorative wear-resistant surface of a floor or wall. The type and quantity of adhesive used to secure the covering to a base does not affect the rupturable characteristics of the floor covering of my invention to any substantial extent.

While I have described and illustrated a preferred embodiment of my invention, it will be understood my invention is not limited thereto since it may be otherwise embodied within the scope of the following claim.

I claim:

As a new article of manufacture, a hard surface floor and wall covering which comprises a decorative and wear-resistant surface, a unitary, partible, felted, fibrous stratum integrally united with said wear-resistant surface and serving as a backing therefor, the fiber constituents of said stratum being substantially uniformly felted throughout the thickness thereof, and an alkyd resin obtained by the reaction of an aliphatic dibasic acid containing 14 to 30 carbon atoms, castor oil, and glycerol, said resin uniformly permeating the fibrous stratum, said stratum carrying said resin possessing a tensile strength within the range of 3 to 30 pounds as determined by the "Scott" test, said resin being the only impregnant for said stratum and being present in an amount by weight falling within the range of 25% to 30% of the weight of the dry saturated fibrous stratum and being dispersed substantially uniformly throughout the mass of the fibrous stratum to render the fibrous stratum substantially water-resistant and to strengthen said stratum to prevent its separation into laminae when exposed to traffic conditions but not completely filling the interstices of said stratum whereby the stratum may be ruptured to permit removal of the floor covering from a base to which it is adhesively secured.

WARREN STUBBLEBINE.

#### REFERENCES CITED

The following references are of record in the file of this patent:

#### UNITED STATES PATENTS

| Number    | Name      | Date          |
|-----------|-----------|---------------|
| 2,272,144 | Allen     | Feb. 3, 1942  |
| 2,274,916 | Adams     | Mar. 3, 1942  |
| 2,295,070 | Allen     | Sept. 8, 1942 |
| 2,316,746 | Stallinge | Apr. 13, 1943 |
| 2,318,272 | Weigle    | May 4, 1943   |

**Certificate of Correction**

August 22, 1950

Patent No. 2,519,410

**WARREN STUBBLEBINE**

It is hereby certified that error appears in the printed specification of the above numbered patent requiring correction as follows:

Column 1, line 53, for the word "is" before "not" read *if*; column 3, line 54, for "in" after "invention" read *is*;

and that the said Letters Patent should be read as corrected above, so that the same may conform to the record of the case in the Patent Office.

Signed and sealed this 7th day of November, A. D. 1950.

**[SEAL]**

**THOMAS F. MURPHY,**  
*Assistant Commissioner of Patents.*